

Oct. 28, 1941.

M. L. STRAWN

2,260,351

METHOD OF FORMING BILLETS

Original Filed Feb. 8, 1937



INVENTOR  
Marion L. Strawn  
By Parker, Carlson, Pitzer & Hubbard  
ATTORNEYS

## UNITED STATES PATENT OFFICE

2,260,351

## METHOD OF FORMING BILLETS

Marion L. Strawn, Rockford, Ill., assignor to The  
Ingersoll Milling Machine Company, Rockford,  
Ill., a corporation of Illinois

Application February 8, 1937, Serial No. 124,640  
Renewed March 21, 1940

1 Claim. (Cl. 29—160.4)

The invention relates to metal billets, commonly known as wire bars, and to an improved method of making the same.

In making wire of copper or the like, the general procedure consists of casting a wire bar or billet, passing the wire bar through a series of rolls to reduce its cross section by elongating the same, then finally extruding the elongated blank through suitable wire drawing dies.

Preparatory to the rolling and drawing operations, it is desirable to remove from the ends of the cast billet any metal containing slag or other imperfections and avoid any resulting sharp edges which might cause cracks or other imperfections to be formed in the finished wire as an incident to the rolling and drawing operations.

It has heretofore been the practice to cast copper wire bars in either horizontal open face molds or in vertical open top molds. The use of open top molds is desirable in that the area of the surface of molten metal exposed to oxidation is minimized and the metal has a finer crystalline structure. On the other hand, such an open top mold produces a bar with a relatively flat upper end portion which contains impurities and as cast is unsuited for proper entry between the reducing rolls. Heretofore, such bars have been prepared for rolling by first cutting off the oxidized end portion and then swaging the ends into a tapered shape. This swaging or mechanical working creates fractures so that the wire drawn from the swaged metal is apt to be weaker or contain imperfections.

The invention resides in the novel method of preparing metal bars of the above character.

Other objects and advantages of the invention will become apparent from the following detailed description taken in connection with the accompanying drawing, in which

Figure 1 is a side view of a vertically cast wire bar or billet prior to the performance of any shaping operations thereon.

Figs. 2 and 3 are side views of an improved wire bar or billet of the form contemplated by the present invention.

Fig. 4 is an enlarged transverse sectional view along the line 4—4 in Fig. 3.

Fig. 5 is a longitudinal sectional view of one end of the billet illustrating the steps of preparing the same for rolling.

While the invention is susceptible of various modifications and alternative constructions, I have shown in the drawing and will herein describe in detail the preferred embodiment, but it is to be understood that I do not intend to limit

the invention by such disclosure but aim to cover all modifications and alternative constructions falling within the spirit and scope of the invention as expressed in the appended claim.

In accordance with the present invention, a rough vertically cast billet 10 (Fig. 1) of copper or the like is prepared for drawing by fashioning the same to form the novel wire bar or billet 11 exemplified in Figs. 2 and 3. Upon reference to Fig. 1, it will be seen that the rough billet 10 is elongated in form and generally rectangular in cross section (Fig. 4) having generally flat side surfaces 8 and rounded or otherwise beveled longitudinal edges 9 merging therewith. The end 12 of the billet 10, which was uppermost in the casting operation, is oxidized, contains impurities such as slag and is irregular in contour. The crystalline structure of the main body of the billet is fine and homogeneous, however, as compared to a similar billet cast in a horizontal open faced mold, and in addition, the mold may be shaped to round or bevel the longitudinal edges of the billet.

In general, improved vertically cast billets of the novel form contemplated by the present invention have tapered ends free of sharp edges and further have a comparatively homogeneous crystalline structure from end to end without weaknesses due to localized mechanical working. Thus, the finished billet 11 has tapered end portions 13 of truncated pyramidal shape terminating in blunt rounded end surfaces 14 which will enter the rolls properly.

The sides 13a of the pyramidal ends 13 are preferably formed as planar continuations of the corresponding sides 8 of the bar in order first to minimize the amount of metal which is removed from the cast metal blank in forming the finished bar. Secondly, the surfaces 13 automatically cooperate with the rolls by which the size of the billet is reduced to automatically square up the body portion of the billet with reference to the rolls. As a result of this cooperation between the rolls and the tapered end as the latter enters between the rolls, the main body of the billet always is fed into the rolls in the proper angular position. The corner surfaces of the tapered ends are beveled or rounded as best shown at 15 in Fig. 4 and merge with the surfaces 8 so that there are no edges in the finished bar having sufficient sharpness to develop into cracks or other imperfections in the rolling operations.

In accordance with the improved method herein contemplated, the slag end 12 of the wire

bar or billet 11 is fashioned in the desired shape by a machining or metal-removing operation such as milling as distinguished from swaging or other mechanical working processes, so that there will be no localized mechanical working 5 strains in the resultant product. In other words, the wire bar 11 will have a substantially homogeneous crystalline structure from end to end and will, in addition, be free of oxide. Despite the fact that the wire bar is shaped by a metal-removing operation, a minimum amount of metal is cut from the blank in view of the improved pyramid-shaped taper which is preferably used.

Preferably, tapering of the ends and removal 15 of the slag containing metal is effected by removing the metal in a succession of layers by a milling cut. Thus, as shown in Fig. 5, cuts on any one side of the billet are taken along dotted lines 17 parallel to the surfaces 13<sup>a</sup> to be formed 20 so as to remove metal layers 18 and form the tapered end. This method of machining is advantageous in that the number of revolutions 25 of relative rotation between the cutter and the billet in order to form the desired taper is reduced to a minimum. In addition, the layers 19 may be removed simultaneously during removal of the final layers 17. If desired, the surfaces 13<sup>a</sup> and the beveled or rounded surfaces 15 may be formed in the same milling operation. Then, 30 by means of a properly shaped milling cutter, successive layers 19 are removed from the end of the tapered portion until all of the slag containing metal is removed.

The opposite end portion of the billet which is formed in the lower end of the mold, usually with a squared end 18, may be tapered in a similar way in order to remove any so-called cold shots that result from splashing and premature solidification of the molten metal initially discharged into the mold. In this instance, however, only enough metal need be removed from the extreme end of the pyramid to impart the desired shape to the end surface 14 and at the same time insure complete removal of the cold shots.

By leaving such a rounded or generally convex surface 14 on the ends, objectionable flowing 15 of the metal during the rolling operations and the consequent formation of a so-called fish tail at the end of the billet is effectually avoided. The necessity of cutting off part of the end of the reduced billet in the course of rolling and a substantial waste of metal are thus eliminated.

I claim as my invention:

The method of preparing a vertically cast billet for rolling and wire drawing which includes the steps of removing successive parallel layers of metal from the slag end of the billet to form a truncated pyramid with beveled edges, and separately removing successive curved layers of slag containing metal from the end of said pyramid to leave a convexly curved end surface.

MARION L. STRAWN.